

## UNITED STATES PATENT OFFICE.

EUGENE L. MAUPAI, OF NEW YORK, N. Y.

## PROCESS OF DYEING RAW SILK.

No Drawing.

Application filed April 23, 1923. Serial No. 624,177.

*To all whom it may concern:*

Be it known that I, EUGENE L. MAUPAI, a citizen of the United States of America, residing at New York city, New York County, State of New York, have invented certain new and useful Improvements in Processes of Dyeing Raw Silk, of which the following is a specification.

My invention relates to a process of dyeing grege or raw silk (single end, not thrown) with developed or diazo colors, or any colors that can be developed with an alkali, or such developers as are used in conjunction with these dyes, and the invention has for its object to provide an inexpensive and efficient dyeing process whereby to eliminate throwing of the untwisted silk and effect dyeing of the same with diazo or similar developed colors, the invention consisting generally in first dyeing the untwisted silk, then diazotizing it to harden the gum and fixing the color, and then developing it, all as hereinafter more fully described and claimed.

In carrying out my improved process, I first impregnate the silk in a bath containing the desired diazo dye, or any developed color, with the addition of approximately 5% to 10% acetic acid, or any acid commonly used in dyeing. Thereafter the silk is washed in a bath of cold water. I then subject the silk to a diazotizing bath, consisting of a solution of cold water and approximately 3% to 5% of sodium nitrite and about 5% of sulphuric or similar acting acid per weight of material used; for certain colors the percentage is decreased or increased. This latter step produces a hardening of the cereaceous or gummy substances and fixes the colors.

Thereafter the silk is thoroughly washed in cold water, and it is then subjected to an alkali developing bath consisting of approximately 5% to 10% of sal soda or any other developer commonly used with developed colors, such as beta naphthol.

I then again wash the silk in either cold

or warm water. It is then dried and woven and may be degummed while in the piece.

By my improved process I am able to 50 eliminate throwing and thereby dye colors fast to boiling off and bleaching on single end grege, which so far as I am aware has heretofore never been accomplished.

What I claim and desire to secure by Letters Patent is:—

1. The process of treating raw untwisted silk, which consists in first dyeing it, then diazotizing it to harden the gum in the silk and fix the color, and then subjecting it to a developing solution.

2. The process of treating untwisted or grege silk, which consists in first impregnating the silk in a diazo dye, then washing the silk, then impregnating the silk in a diazotizing bath, then again washing the silk, and then subjecting it to an alkali developing bath.

3. A step in the process of dyeing grege or untwisted silk, which consists in initially dyeing it with diazo colors, and then in a single operation hardening the gummy substances in the silk and fixing the colors.

4. The process of dyeing untwisted raw silk, which consists in first dyeing the silk with diazo or similar dyes, then washing the silk, then impregnating the silk in a diazotizing bath comprising water and sulphuric acid and sodium nitrite, then again washing the silk, and finally subjecting the silk to a developing bath.

5. The process of dyeing untwisted raw silk, which consists in first impregnating the silk in a bath containing a suitable diazo dye with the addition of acetic acid, then washing the silk, then subjecting it to a diazotizing solution of sodium nitrite and sulphuric acid to harden the gummy substances in the silk, then washing the silk, then immersing it in an alkali developing bath, then again washing the silk, and then drying weaving and degumming the silk.

EUGENE L. MAUPAI.